

A. J. PARRISH.  
PROCESS OF MAKING MONOLITHIC PAVEMENTS.  
APPLICATION FILED AUG. 1, 1917.

1,347,654.

Patented July 27, 1920.



WITNESSES  
E. H. Gallagher  
H. J. Bosse

INVENTOR  
ALAN JAY PARRISH  
BY *Allen J. Parrish*  
ATTORNEYS

# UNITED STATES PATENT OFFICE.

ALAN JAY PARRISH, OF PARIS, ILLINOIS.

## PROCESS OF MAKING MONOLITHIC PAVEMENTS.

1,347,654.

Specification of Letters Patent. Patented July 27, 1920.

Application filed August 1, 1917. Serial No. 183,907.

To all whom it may concern:

Be it known that I, ALAN JAY PARRISH, a citizen of the United States, and a resident of Paris, in the county of Edgar and State 5 of Illinois, have invented an Improvement in Processes of Making Monolithic Pavements, of which the following is a specification.

My invention relates to improvements in 10 processes for making monolithic pavements, and it consists in the steps herein-after described and claimed.

In the construction of brick pavements, especially those which are designed for 15 making roadways, the practice heretofore has been to provide a base having a cushion of sand and to embed the bricks in the sand, either filling the spaces between the bricks with sand or grouting the bricks with 20 a cement filler. Pavements built in this way are liable to rapid disintegration for the reason that it is impossible to keep the water from entering between the bricks. This may wash away portions of the sand 25 and cause the bricks to settle, thus rendering the roadway rough and uneven. The frost may also cause the buckling of the roadway. Furthermore, bricks or blocks laid in a cushion of sand have some of the sand 30 forced up from the bottom between the bricks. This prevents the filling of the space between the bricks with cement clear to the bottom and makes only a bond from the surface of the brick down a portion of 35 its depth. When traffic comes on the brick the bond will break, since it is not embedded or bonded at the bottom.

The purpose of the present invention is to 40 provide a monolithic construction in which a base of concrete is provided, the bricks being set in the plastic concrete and pressed and then the spaces between the bricks filled with cement filler, so that when the cement and concrete harden the whole forms a rigid 45 monolithic structure which is not liable to disintegrate as in the case of the construction with the sand cushions.

A further object of my invention is to 50 provide a construction which may be made rapidly and which does not require the hardening of the base before laying the bricks.

Other objects and advantages will appear 55 in the following specification, and the novel features of the invention will be particularly pointed out in the appended claims.

My invention is illustrated in the accom-

panying drawing which is a perspective view of a portion of a monolithic pavement constructed according to my invention.

In carrying out my invention I make use 60 of forms, such as that shown at 1 in the drawing, which are placed at the sides of the roadway. A layer of concrete 2 is first deposited on the roadway. The consistency of this concrete is such that when a portion 65 of it is squeezed between the hands it will retain its shape. This layer is deposited to a desired depth and then is struck off by means of a templet or strike plate in a shape to conform to the curvature of the 70 roadway.

A thin film 3 of a mixture of sand and cement is now placed over the concrete base while the latter is in its plastic condition. The water from the plastic concrete base 75 will be drawn up by capillary attraction into the mixture of sand and cement so as to wet it. The bricks 4 are now laid directly on the layer of sand and cement, which layer tends to form a cement mortar. The 80 bricks are now rolled with a roller so as to bring them to a smooth surface. Immediately after the bricks have been rolled they are grouted with a cement filler, which enters the spaces between the bricks and which 85 firmly binds them together when the cement has set. In the construction of brick pavements it has heretofore been customary to wait until the base has set before proceeding further with the construction. I have 90 found that a plastic concrete base having a thin coating of the cement mortar made by mixing dry cement and sand as described may be immediately utilized as a base by placing the bricks thereon while the base and 95 its thin coating of mortar are in a plastic condition. Furthermore the bricks may be immediately walked on, as for the purpose of rolling them and grouting them. The bricks sink to a certain degree in the plastic concrete, but this is an advantage rather than a detriment, because of the fact that it forces the mortar up between the lower parts of adjacent bricks, thereby forming a 100 firm anchorage for the bricks.

The construction defined above provides an ideal pavement. Ordinarily vitrified bricks are used and after considerable use it will be found that the bricks are well bound together. In fact, where any breakage takes place, it will be found that the break will be through the brick itself, 110

rather than along the edges of the brick where one would naturally suppose that the break would come. In other words the construction is virtually monolithic.

5 I claim:

1. The herein described process of making monolithic pavements which consists in depositing a layer of plastic concrete, striking off the concrete to a desired shape, adding a thin coating of sand and cement mixed dry to the concrete while the latter is in its plastic condition, placing the bricks on the coating while the latter and the concrete are in a plastic condition, pressing the bricks to bring the top of the latter to a smooth surface while the concrete and said coating are in a plastic condition, and grouting the bricks with a cement filler capable of hardening and firmly binding the bricks together.
- 10
- 15

with a cementitious binding material.

2. The herein described process of making monolithic pavements which consists in depositing a layer of plastic concrete, striking off the concrete to a desired shape, adding a thin coating of sand and cement mixed dry to the concrete while the latter is in its plastic condition, placing the bricks on the coating while the latter and the concrete are in a plastic condition, pressing the bricks to bring the top of the latter to a smooth surface while the concrete and said coating are in a plastic condition, and grouting the bricks with a cement filler capable of hardening and firmly binding the bricks together.
- 20
- 25
- 30

ALAN JAY PARRISH.